

Jan. 15, 1946.

H. H. DUERR ET AL.

2,393,027

MULTILAYER REVERSAL COLORFILM AND METHOD OF PROCESSING THE SAME

Filed Nov. 6, 1942



INVENTORS  
Herman H. Duerr  
Herbert W. Morreall, Jr.  
BY  
Henry W. Coughlin  
ATTORNEY

## UNITED STATES PATENT OFFICE

2,393,027

MULTILAYER REVERSAL COLOR FILM AND  
A METHOD OF PROCESSING THE SAMEHerman H. Duerr and Herbert W. Morreall, Jr.,  
Binghamton, N. Y., assignors to General Aniline  
& Film Corporation, New York, N. Y., a corpo-  
ration of Delaware

Application November 6, 1942, Serial No. 464,715

9 Claims. (Cl. 95—2)

The present invention relates to multilayer reversal colorfilm having a high speed and fine grain, amenable to control of the color balance and to a method of processing the same.

Multilayer colorfilm is known in which the three layers sensitive respectively to red, green and blue light, contain color formers which are fast to diffusion. A method of processing such film by the reversal method involving the formation of dye images by reaction of the color formers in the emulsion layers with the oxidation products of an aromatic amino developer, is also known, as may be appreciated from a reference to U. S. P. 2,179,234. While such film and the processing of the same by the method of said patent leads generally to satisfactory results, the film is not entirely free from objections.

The cyan image is the key image in subtractive color photography and it is therefore essential that the layer destined to contain such image be amenable to processing to produce a strong image. This in turn means that the film must have a satisfactorily high speed. In order to obtain the desired speed, resort must be had to the usual powerful red sensitizers. It is a peculiarity of the color formers utilized to produce cyan dye images that for the most part they have a tendency to displace the sensitizers from the silver halide grains. Since the ability of a sensitizer to adequately perform its function depends upon its absorption by the silver halide grains, a displacement of the sensitizers from the grains by the color formers leads to emulsion layers of low speed. While some of the red sensitizers are compatible with cyan color formers, and may sensitize properly when present in the layer with cyan color formers, nevertheless the number of such sensitizers is relatively restricted.

There are many color formers capable of producing dye images upon reaction with the oxidation products of aromatic primary amino developers. However, the number of color formers which are capable of permitting the introduction of groups rendering the color formers fast to diffusion without detrimentally influencing the speed or color absorption of the resulting dyes, is relatively small. Therefore there is a definite limitation placed upon the art, first as regards color formers when utilizing film to be produced according to U. S. P. 2,179,234, and second as regards sensitizers.

This limitation in the selection of the sensitizers and the color formers is not the only problem which confronts the art when working according to said patented procedure. In the patented procedure, all of the dye images are produced in one development step. This means that the reaction leading to the dye images in the

three sensitive layers must produce satisfactory dye images in the single developing step, and precludes a possibility of adjusting the reaction to take care of irregularities which may be inherent particularly in the red-sensitive layer. Inasmuch as it is difficult to obtain an absolute uniformity in all of the layers so that the reaction producing the dye image leads to images having a proper color balance, a further problem is presented by the fact that where the color formers are located in the film itself, compensation for irregularities cannot be effected by adjusting the time of development.

We have now found that wide latitude in the selection of color formers and sensitizers can be insured with the production of a film giving the desired color balance by producing a film in which the color formers for the yellow and magenta images are located in the blue- and green-sensitive layers, respectively, whereas no color former is located in the red-sensitive layer, and separately processing the red-sensitive layer so as to permit an adjustment of the time of development. The production of such film and the processing of the same constitute the purposes and objects of the present invention.

The invention will be more readily understood by reference to the accompanying drawing which discloses in section a film of the type contemplated herein. Figure 1 of the drawing discloses one modification, and Figure 2 a different modification.

Referring to Figure 1, reference numeral 1 discloses an antihalation layer removable in an alkaline solution or decolorizable in the developing process. A suitable antihalation layer in the first category consists of an alkali-soluble resin such as is described in U. S. P. 2,161,788 and containing dyes such as are mentioned in U. S. P. 2,147,112. An antihalation layer falling within the second category is a colloidal silver layer such as that described in U. S. P. 2,220,187. 6 represents a film base on which are supported five superimposed layers, three layers of which are gelatino-silver halide emulsion layers. Layer 5 is a red-sensitive silver halide layer which contains no color component. Due to the absence of the color component, one may use any of the known powerful sensitizers for red without any fear of a detrimental action on the sensitizer. Layer 3 is a green-sensitive silver halide emulsion layer containing a non-diffusing magenta color component. Satisfactory color components for the magenta image are the non-diffusing components described in U. S. Patents 2,178,612 and 2,179,238. Examples of such components are the condensation products of meta-amino-phenyl-methyl-pyrazolone, and the mixed polymer of

vinyl chloride and maleic acid anhydride, para-(hydroxy - naphthoyl - amino) - 1 - phenyl - 3 - methyl-5-pyrazolone and the like. Layer 1 is a blue-sensitive silver halide emulsion layer containing a non-diffusing yellow color component. Satisfactory components for this layer are the non-diffusing components described in U. S. Patents 2,179,238 and 2,224,329. Specific examples of such components are terephthaloyl-bis-acetic acid anilid-p'-carboxylic acid and the like. Interposed between the blue-sensitive layer 1 and the green-sensitive layer 3 is a yellow filter layer which may be of colloidal silver or which may be of a yellow dyestuff of the type contemplated in U. S. P. 2,187,731. Interposed between the green-sensitive layer 3 and the red-sensitive layer 4 is a third gelatin layer which may, however, be omitted without any particular sacrifice of results.

The multilayer film may be processed by exposing the same to a colored object and developing the film to a negative in a developer which will not couple with the components in the blue- and green-sensitive layers. For this purpose one may utilize the amidol developer described in U. S. P. 2,179,234. The red-sensitive bottom layer is then exposed through the base to red light without affecting the green-sensitive and blue-sensitive layers. The re-exposed red-sensitive layer is then color-developed in a developer containing a cyan color component which of course must be one which is diffusing rather than non-diffusing. Suitable cyan developers are those mentioned in U. S. P. 2,191,502 and 1,969,452. Examples of such developers are:

|                                              |     |    |
|----------------------------------------------|-----|----|
| Sodium sulfite (anh.)                        | g.  | 5  |
| Potassium carbonate                          | g.  | 30 |
| Diethyl - p - phenylenediamine hydrochloride | g.  | 3  |
| Water                                        | l.  | 1  |
| 2,3,4-trichlor-alpha naphthol                | g.  | 2  |
| Dissolved in ethyl alcohol                   | cc. | 25 |

or

|                                              |     |    |
|----------------------------------------------|-----|----|
| Sodium sulfite                               | g.  | 40 |
| Sodium carbonate                             | g.  | 60 |
| Diethyl - p - phenylenediamine hydrochloride | g.  | 3  |
| 2,4 dichloro $\alpha$ -naphthol              | g.  | 2  |
| In acetone                                   | cc. | 60 |
| Water to make                                | l.  | 4  |

In lieu of the naphthols mentioned in the above formulae, one may employ  $\alpha$ -naphthol and pentabrom- $\alpha$ -naphthol or meta-hydroxydiphenyl. Following the formation of the cyan color image, the blue-sensitive top layer and green-sensitive middle layers are simultaneously exposed to blue-green light and developed in a color-forming developer which is free from color-forming substances. Developers of this type are paraphenylenediamine developers, and we have found that satisfactory results may be obtained when using the developer mentioned in U. S. P. 2,179,234. By this step a yellow image is formed in the blue-sensitive top layer and a magenta image in the green-sensitive middle layer. The multilayer film is now subjected to bleaching in a ferricyanide bleaching bath to effect a removal of both the positive and negative silver, after which it is fixed, washed and dried. Suitable silver-bleaching baths are those referred to in U. S. P. 2,113,329. Examples of silver bleaching baths which we have found to be particularly effective are the following:

|                        |      |      |
|------------------------|------|------|
| Potassium ferricyanide | gms. | 10   |
| Water to               | cc.  | 1000 |
| or                     |      |      |
| Cupric chloride        | gms. | 20   |
| Potassium bromide      | gms. | 10   |
| Water to               | cc.  | 1000 |
| or                     |      |      |
| Ammonium bromide       | gms. | 75   |
| Iodine (cryst.)        | gms. | 3    |
| Water to               | cc.  | 1000 |

A fixing bath of 10% sodium thiosulfite may be used. The film is now ready for projection.

It will be appreciated that since color is introduced into the red-sensitive bottom layer by a separate development step, and since the silver halide which is responsible for color formation is exposed by a separate step, it is possible to control the color balance by adjusting the re-exposure and developing time of the red-sensitive layer. The advantages of this processing over the processing disclosed in U. S. P. 2,179,234 will become immediately apparent.

It is of course not essential that one adhere strictly to the sequence of steps which have been just related. Thus, we have worked up the film by re-exposing the two top layers with blue-green light following the black-and-white development and have then developed these in a color-forming developer free from color components, such as that mentioned above. After this, the cyan layer may be exposed and processed as previously described. Furthermore, it is not necessary to employ light for re-exposure of the various layers. Thus in either of the procedures outlined, the two top layers may be simultaneously fogged by exposure with minus red light and then color developed while the red-sensitive bottom layer may be chemically fogged and then color developed with a developer containing a cyan color component. Suitable chemical fogging agents are those disclosed in U. S. P. 2,159,466. An example of a fogging agent which we have found to give particularly good results is:

|                     |     |      |
|---------------------|-----|------|
| Water               | cc. | 1000 |
| Glacial acetic acid | cc. | 5    |
| Thiosinamine        | gr. | 0.4  |

One may utilize, in place of the thiosinamine in this example, n-phenyl thiourea, N-N diethyl-N'-allyl thiourea, N-N diethano-N'-phenylthiourea and the like.

It will be observed from a reference to Figure 2 that the film thereof is similar to that of Figure 1 in so far as layers 1-3 inclusive are concerned. The film differs from that of Figure 1 in that a second yellow filter layer, 4a, is interposed between the green-sensitive emulsion layer 3 and the red-sensitive emulsion layer 5, and that an antihalation layer of colloidal silver, 6a, is interposed between the base 6 and the red-sensitive emulsion layer 5. The red-sensitive emulsion layer 5 is similar to that of Figure 1 in that it is free from color-forming components. The color-forming components mentioned for use in the blue- and green-sensitive emulsion layers of Figure 1 may likewise be used in the film of Figure 2.

The film of this figure is processed by exposing it to a colored object and developing it to a black-and-white negative in a developer such as amidol, the oxidation products of which do not couple with the color components in the blue- and green-sensitive layers. The bottom layer is then ex-

posed to white light and due to the presence of a colloidal silver antihalation layer which is reddish-brown in color, together with the yellow filter layer between the cyan and magenta layer, exposure of the magenta layer is prevented. The red-sensitive layer is then developed in a color developer containing a cyan color-coupling component of the type described above. Here, again, color balance can be assured by correlating the time of exposure with the time of development. The blue-sensitive top layer and the green-sensitive intermediate layer are now exposed with white light and developed in a color-forming developer free from color-forming substances. The developer mentioned above may also be employed in this instance. Finally, the film is bleached with a silver bleaching bath of the type recommended above and after fixing is washed and dried. The film is then ready for projection and it will be found to have a proper color balance.

It will be seen that working by the method claimed, any red sensitizer suitable for the sensitizing of a silver halide emulsion to the red region of the spectrum may be utilized, inasmuch as no color formers are present in the red-sensitive layer and hence one may disregard the fact that cyan color formers normally have a greater affinity for silver halide grains than do red sensitizers. Similarly, by utilizing a diffusing color component for production of the cyan image, the number of possible color formers which the art may select is greatly enhanced, since one need not pay any particular attention to the necessity of incorporating groups into the color former which would render the same fast to diffusion. Finally, by permitting a separate development of the red-sensitive layer, the time of development may be so correlated with the other factors as to insure a proper color balance between the various dye images.

Modifications of the invention will occur to persons skilled in the art and we therefore do not intend to be limited in the patent granted, except as required by the claims and the prior art.

We claim:

1. The method of producing multicolor photographs which comprises exposing a multilayer film comprising a base, a red-sensitive layer on said base free from color-forming components, a green-sensitive layer above said red-sensitive layer, containing a nondiffusing color component for color forming development for the magenta image, a blue-sensitive outer layer containing a non-diffusing color component for color forming development for the yellow image, and a yellow filter interposed between the blue-sensitive and green-sensitive layers, developing the film to a black-and-white negative in a developer whose oxidation products do not couple with the color formers in the emulsion layers, rendering developable the silver halide of one of the groups of layers comprising the blue-sensitive and green-sensitive layers on the one hand and the red-sensitive layer on the other hand and without rendering developable the silver halide of the other group, color developing the silver halide so rendered developable, rendering the previously untreated silver halide developable and color developing the same, the red-sensitive layer being color-developed in a color developer containing a cyan color component.

2. The process as defined in claim 1 in which all of the positive and negative silver is removed after the final color-developing step.

3. The method of producing multicolor photographs which comprises exposing a multilayer film comprising a base, a red-sensitive layer on said base free from color forming components, a green-sensitive layer above said red-sensitive layer, containing a nondiffusing color component for color forming development for the magenta image, a blue-sensitive outer layer containing a nondiffusing color component for color forming development for the yellow image, and a yellow filter interposed between the blue- and green-sensitive layers, developing the film to a black-and-white negative in a developer whose oxidation products do not couple with the color formers in the emulsion layers, re-exposing the silver halide of the blue-sensitive and green-sensitive layers without exposing the silver halide of the red-sensitive layer, color developing the exposed silver halide, rendering the previously unexposed silver halide in the red-sensitive layer developable, and developing the same in a color developer containing a cyan color component.

4. The process as defined in claim 3 wherein the red-sensitive layer is rendered developable by chemical fogging agents.

5. The process as defined in claim 3 wherein the red-sensitive layer is rendered developable by re-exposure.

6. The process as defined in claim 1 wherein the red-sensitive layer is re-exposed with red light and the yellow-and-green-sensitive layers are re-exposed with blue-green light.

7. The process of producing multicolor photographs from a multilayer film comprising a base, an antihalation layer of colloidal silver on said base, a red-sensitive emulsion layer free from color components on said antihalation layer, a yellow filter layer on said red-sensitive layer, a green-sensitive emulsion layer containing a non-diffusing color component for color forming development for the magenta image on said yellow filter layer, a yellow filter layer on said green-sensitive layer, and a blue-sensitive emulsion layer containing a nondiffusing color component for color forming development for the yellow image on said second yellow filter layer, which comprises exposing said film to a colored object, developing the film to a black-and-white negative in a developer the oxidation products of which do not couple with the color components in the emulsion layers, re-exposing the red-sensitive layer with white light while insuring that the anti-halation layer and the filter layer between the green-and red-sensitive emulsion layers prevents exposure of the green-sensitive and blue-sensitive emulsion layers, color-developing the re-exposed red-sensitive emulsion layer in a color developer containing a cyan color former, rendering developable the blue- and green-sensitive emulsion layers and developing the same in a color developer and submitting the film to the action of a silver-bleaching agent to remove all of the negative and positive silver plus the colloidal silver in the filter and anti-halation layers.

8. The process as defined in claim 1 wherein the blue- and green-sensitive layers are rendered developable by chemical fogging agents.

9. The process as defined in claim 1 wherein the blue- and green-sensitive layers are rendered developable by re-exposure.

HERMAN H. DUERR.

HERBERT W. MORREALL, JR.